# EUROPEAN PATENT APPLICATION

(11) **EP 1 502 965 A1**
(43) Date of publication of application: **02.02.2005**
(21) Application number: 04466021.5
(22) Date of filing: 29.07.2004
(51) Int. Cl.: C22C 9/04

(54) **Free cutting brass alloy**

(30) Priority: 01.08.2003 CZ 20032094
(71) Applicant: Kovohute Celakovice, a.s., 250 88 Celakovice (CZ); VUK Panenske Brezany, s.r.o., 250 70 Odolena Voda (CZ)
(72) Inventor: Strachovsky, Antonin, 250 88 Celakovice (CZ); Faltus, Jiri, 152 00 Praha 5 (CZ)
(74) Representative: Belfin, Vladimir

(57) **Abstract**

The free cutting brass alloy on the basis of alloy Cu-Zn-Bi is designed primarily for hot and cold moulding, especially for manufacturing rods by cold drawing, and contains 55,0 % to 75,0 % by weight of copper, 0,5 % to 4,0 % by weight of bismuth, zinc residue and incidental tramp elements and impurities, such as 0,001 to 0,2 % by weight of lead and/or 0,001 to 0,3 % by weight of phosphor, 0,001 to 3,0 % by weight of silicon, 0,001 % to 2,0 % by weight of tin, a max. of 0,1 % by weight of aluminum, a max. of 0,4 % by weight of iron, a max. of 0,3 % by weight of nickel and a max. of 0,5 % by weight of other tramp elements on the whole.

## Description

### Field of the Invention

The invention concerns a free cutting brass alloy for heat and could moulding, primarily for manufacturing of rods by cold drawing.

### Background of the Invention

The current free cutting brasses, also known as screw brasses, are mostly Cu-Zn-Pb alloys and usually contain 57,0 to 60,0 % by weight of copper, 1,0 to 4,5 % by weight of lead and zinc residue. From these alloys are manufactured rods, tubes, profiles and wires by hot working. During the subsequent cutting operation, a fragile chip occurs due to the presence of lead.

However, a harmful effect of lead on human health is a disadvantage of these brasses that significantly limits their applicability. Thus, they can not be used for manufacturing of indoor installation elements and components for drinking water as valves, water meters, various pipe unions and etc. because lead in these brasses is at long-term functions released into water medium. This causes an increase in content of lead in drinking water. The higher the content of lead in the brass, the higher quantity of it is released into water.

This disadvantage is largely eliminated by a brass known from the published patent application CZ PV 1999-4367 designed primarily for working and subsequent cutting operation. The brass contains 57,0 to 60,0 % by weight of copper, 0,5 to 2,5 % by weight of bismuth and zinc residue. It may also contain lead, namely either as a tramp element or an alloying element when together with bismuth creates an addition to break a chip. Depending on the required need and purpose it may further also contain 0,15 to 0,3 % by weight of phosphor, incidentally a maximum of 0,1 % by weight of aluminum, a max. of 0,4 % by weight of iron, a max. of 0,3 % by weight of nickel, a max. of 0,1 % by weight of tin or a max. of 0,2 % by weight of other tramp elements on the whole.

Nevertheless, neither this known workable brass fulfills all requirements, especially from the material structure and properties point of view resulting from requirements e.g. in automobile industry. It is not appropriate for other applications where significantly higher contents of copper and other alloying and tramp elements are required, namely because of its better drawability.

### Summary of the Invention

The mentioned above disadvantages of the current technology have been largely eliminated by use of free cutting brass alloy on the basis of Cu-Zn-Bi alloy, designated especially for cold drawing, according to the invention. The principle of the invention consists in the fact, that the free cutting alloy brass contains 55,0 % to 75,0 % by weight of copper, 0,5 to 4,0 % by weight of bismuth as an exclusive addition, chip-breaking addition, zinc residue and incidental tramp elements and impurities.

In contrast with so far known workable brasses that have generally two phases - so called "alpha" and "beta", the free cutting brass alloy according to the invention is a one-phase brass. It consists of only alpha phase with all positive implications on its properties and can be widely applied in various areas in industry.

The principle of the invention lies further in the fact that the fee cutting brass alloy may also contain lead. However, unlike so far known workable brasses, lead is here only as a tramp element in the quantity of 0,001 to 0,2 % by weight.

An alternative modification of the free cutting brass alloy according to the invention where there is a requirement on a higher corrosion resistance, may further contain 0,05 to 0,3 % by weight of phosphor.

According to the invention, the free cutting brass alloy may also contain 0,01 to 3,0 % by weight of silicon, incidentally 0,01 to 2,0 % by weight of tin, a max. of 0,1 % by weight of aluminum, a max. of 0,4 % by weight of iron, a max. of 0,3 % by weight of nickel and a max. of 0,5 % by weight of other tramp elements on the whole.

The advantage of the free cutting brass alloy according to the invention is the fact that although this brass is unlike the current brasses practically leadless one, its workability is practically equal to common alloys Cu-Zn-Pb, such as e.g. CuZn40Pb2. At the same time, in contrast with other known so called leadless workable brasses, its drawability has been significantly improved while preserving its good formability. It can be processed by common way, such as casting, extrusion, rolling and unrolling of extrusions, cold drawing, straightening, sanding, drop forging or hot forging.

### Examples of Modifications of the Invention

### Example 1

According to this example of the invention, the free cutting brass alloy contains 70,47 % by weight of copper, 1,24 % by weight of bismuth and zinc residue.

### Example 2

In the second example, the free cutting brass alloy contains 60, 97 % by weight of copper, 1,51 % by weight of bismuth, 0,009 % by weight of tin, 0,071 % by weight of lead, 0,003 % by weight of aluminum, 0,006 % by weight of iron, 0,022 % by weight of nickel, 0,018 % by weight of phosphor, less than 0,01 % by weight of silicon, zinc residue.

According to these two examples, the free cutting brasses were manufactured in a channel-type furnace. The both casts were prepared from copper Cu99,5, zinc Zn99,5, bismuth Bi99,9 and foundry alloy CuP10. From the casts, ingots with a diameter of 184 mm were cast by stationary casting into copper water-cooled moulds. From these ingots dimension stock in a length of 770 mm were then prepared and directly extruded on extrusions in a diameter of 18,5 mm. The extrusion was conducted at a temperature of 720 to 740 °C at a leaving velocity of 3 to 4,5 m/min.. After leaving the press, extrusions were coiled into circles in a diameter of 1,2 m. These extrusions were then straightened on prismatic cylinders, then cold drawn into a diameter of 18,0 mm and straightened and cut into the required length of 3,0 m.

The reached mechanical properties of both types of the brasses according to the examples are specified at the following table:

| | Rp0,2 [MPa] | Rm[MPa] | A5 [%] | HB |
|---|---|---|---|---|
| 1. Example | 156 + 12 | 438 + 1 | 31 + 6 | 107 + 0,4 |
| 2. Example | 153 + 7 | 438 + 5 | 36 + 1 | 99,5 + 0 |

### Field of the Aplication

The free cutting brass alloy according to the invention can be widely used primarily for forgings, solid or hollow rods and other profiles that are further designed for cutting operation.

## Claims

1. Free cutting brass alloy on basis of alloy Cu-Zn-Bi, designed primarily for cold drawing, **characterized by** the fact, that contains 55,0 to 75,0 % by weight of copper, 0,5 to 4,0 % by weight of bismuth, zinc residue and incidental tramp elements and impurities.

2. Free cutting brass alloy according to the claim 1, **characterized by** the fact, that further contains 0,001 to 0,2 % by weight of lead.

3. Free cutting brass alloy according to at least one of above stated claims, **characterized by** the fact, that further contains 0,001 % to 0,3 % by weight of phosphor.

4. Free cutting brass alloy according to at least one of above stated claims, **characterized by** the fact, that further contains 0,001 % to 3,0 % by weight of silicon.

5. Free cutting brass alloy according to at least one of above stated claims, **characterized by** the fact, that further contains 0,001 % to 2,0 % by weight of tin.

6. Free cutting brass alloy according to at least one of above stated claims, **characterized by** the fact, that further contains max. 0,1 % by weight of aluminum, max. 0,4 % by weight of iron, max 0,3 % by weight of nickel and max. 0,5 % by weight of other tramp elements on the whole.
